

May 4, 1926.

E. J. GUAY

1,583,592

INDURATED MATERIAL AND METHOD OF MANUFACTURING THE SAME

Filed August 15, 1921

Fig. 1.



Fig. 2.



Fig. 3.



Fig. 4.



Inventor,  
Emile J. Guay,  
by Abbott Davis  
His Attorney.

## UNITED STATES PATENT OFFICE.

EMILE J. GUAY, OF LYNN, MASSACHUSETTS, ASSIGNOR TO GENERAL ELECTRIC COMPANY, A CORPORATION OF NEW YORK.

## INDURATED MATERIAL AND METHOD OF MANUFACTURING THE SAME.

Application filed August 15, 1921. Serial No. 492,624.

To all whom it may concern:

Be it known that I, EMILE J. GUAY, a citizen of the United States, residing at Lynn, in the county of Essex, State of Massachusetts, have invented certain new and useful Improvements in Indurated Materials and Methods of Manufacturing the Same, of which the following is a specification.

The present invention relates to indurated material made from spinnable textile material and an adhesive binder and to the manufacture of such material.

The object of the invention is to provide an improved indurated material of this type and an improved method of manufacturing the same whereby there is obtained an indurated product possessing physical properties which make it superior to similar products manufactured by methods heretofore in use. Particularly is this true where the indurated material is to be put to uses requiring great strength coupled with elasticity, that is, ability to deflect without breaking. One extensive application for indurated material of this character and an application where great strength coupled with elasticity are of highest importance is for gear wheels, such gear wheels being known as non-metallic or noiseless gear wheels. The life of non-metallic or noiseless gear wheels made of indurated material formed from spinnable textile material and an adhesive binder is directly proportional to the strength of the indurated material and its ability to deflect under load, (other things being equal) and by tests I have found that indurated material made by my improved method is much stronger and more flexible than similar material made by other methods in common use. As a result gear wheels manufactured from indurated material made in accordance with my invention will have a life substantially longer than gear wheels manufactured from similar material made by other known methods.

According to my method I take pieces of spinnable textile material comprising hard twisted threads such as a suitable grade of canvas or cotton duck for example, and stack them one on another with a thin layer or covering of adhesive binder in dry form between successive pieces. When the textile material is in the form of woven fabric, the pieces are stacked preferably with the warp of successive pieces at a right angle to each

other, since such cloth is stronger in one direction than the other and by stacking them in this manner a mass equally strong in both directions results. According to one embodiment of my invention, in forming a stack I take a supporting plate which may be made of metal, sprinkle a thin layer of powdered adhesive over its surface, place a piece of fabric thereon, sprinkle a thin layer of powdered adhesive on its upper surface, place another piece of fabric on the first piece with its warp at a right angle to the warp of the first piece, sprinkle a thin layer of powdered adhesive on it and continue in this manner until a stack is formed having the desired number of layers. A metal plate similar to the bottom plate may be then placed on the top of the stack after which the entire built-up structure is placed in a press and subjected to heavy pressure. I may use an hydraulic press and have found pressure of from 600 lbs. per sq. inch to 900 lbs. per sq. inch satisfactory. While the stack is held under pressure, and preferably while it is still in the press, I subject it to heat to fuse the adhesive and cause it to permeate the layers of fabric. The extent and intensity of the heating will depend upon the character of the adhesive material and can be readily determined by experiment. After the heating is completed, the stack is cooled while still held under pressure after which it is removed from the press. I then have an indurated plate or board formed of successive layers of woven fabric held under heavy pressure by the adhesive. As an adhesive I preferably use powdered bakelite, or powdered shellac, but I may use other adhesives which can be obtained in powdered form.

In an indurated material of this character, it is the textile material held under high compression which lends the strength and toughness to it, the adhesive acting only as a binder. The strength and toughness is due to the many fibres held in close contact with each other and the greater the number of fibres thus held the greater the strength and toughness. By the method just described wherein I use adhesive in powdered form and place the textile material under high pressure before the adhesive is fused, the fibres are brought into very close contact so the adhesive when fused is prevented from entering to any great extent between the cot-

ton fibres and particularly between the fibres which form the individual threads, such threads being in substance a bundle of fibres. In the manufacture of indurated material of this character, by methods heretofore in use, the adhesive has, so far as I am aware, been applied to the fabric in liquid form, the adhesive being carried by a suitable solvent, and then dried to drive off the solvent. 10 I have found that by this method the adhesive is carried in around the fibres to a great extent so that when sheets which have been impregnated with a liquid adhesive and dried are compressed, heated and hardened, 15 the individual fibres contact directly with each other to a less degree than is the case with my improved method. I consider therefore the use of adhesive located primarily on the surfaces of the threads, as is the case 20 when the adhesive is used in powdered form, and the compressing of the built up stack prior to any heating or impregnating of the textile material with the adhesive as being important features of my invention. It will 25 be noted that prior to the heating operation, the dry adhesive is located primarily on the surfaces of the individual threads, and when this dry adhesive, such as bakelite, becomes liquefied by the heat, it distributes itself 30 around among the threads to fasten them together. Since at the time, however, the threads are held under compression, the fused adhesive does not saturate all the individual fibres as is the case when a solvent 35 is used, but enters more around the bundles of fibres, thus making a much stronger product.

In the accompanying drawing which is illustrative of my invention, Fig. 1 is a top plan view partly broken away showing one manner of carrying out my method; Fig. 2 is a side elevation of a stack of sheets prior to being compressed; Fig. 3 shows the same stack of sheets between the jaws of an hydraulic press and after they have been compressed, and Fig. 4 shows a block of the finished material.

Referring to the drawing, 5 indicates the lower plate and 6 the upper plate between 50 which are a number of sheets of woven fabric 7, there being a thin covering of adhesive between each of the sheets.

I have made a most satisfactory product from heavy cotton duck and powdered bakelite, and I shall now specifically describe my method when utilizing these materials.

I first place the plate 5, which is preferably a metal plate, upon a suitable support and cover it with a very thin coating of 60 powdered bakelite. This may be sprinkled on by hand or dusted on by a suitable machine. I then place a sheet of cotton duck on plate 5 after which a thin coating of the powdered bakelite is sprinkled on the upper 65 surface of the sheet. Following this I place

a second sheet of duck on the first one, with the warp at a right angle to that of the first sheet, and sprinkle a thin coating of powdered bakelite on it. This is repeated until a stack of the desired height is obtained. 70 With heavy duck I have found that about fifty sheets are required to provide sufficient material for a finished product one inch thick.

After the sheets 7 have been stacked in place I put the top plate 6 on the uppermost one. This plate may be of the same character as the plate 5. The stack of sheets held between plates 5 and 6 are then placed between the jaws of an hydraulic press 75 which are indicated diagrammatically at 8 and 9. These jaws are preferably hollow and are provided with pipes 10 leading to the interior of them so that steam for heating purposes and water for cooling purposes 80 may be admitted. The press is operated to place the stack of material under a pressure of about 700 lbs. per square inch. This brings the fibres of the material into very 85 close contact. Steam is then admitted to the jaws 8 and 9 of the press for the purpose of fusing the bakelite and causing it to stick the sheets of fabric together. The heating is preferably performed gradually. I may first admit low pressure steam of a 90 pressure of about 10 to 20 lbs. (temperature about 240° F.) for about ten minutes. The temperature may then be raised by taking steam of 40 to 50 lbs. pressure (temperature 95 285° to 295° F.) this temperature being 100 maintained for from 10 to 15 minutes. I then admit steam of about 110 lbs pressure (temperature about 345° F.) maintaining 105 this for about two hours or more depending on the thickness of the stack of sheets. During the compression and heating excess of bakelite is squeezed out around the edges of the stack of sheets. The powdered bakelite is dusted on sparingly so there will be little excess the approximate amount to use 110 being readily determined by experiment.

After the heating process is completed the steam is shut off and cooling water admitted through the pipes 10 to cool the material. The pressure is maintained during the cooling and when the desired low temperature is reached the hydraulic press is opened and the finished product removed. It is then 115 ready to be used for any purpose for which it may be found applicable, for example, 120 the making of gear wheels.

A characteristic feature of my invention and one which I consider of great importance is that of having the adhesive material on the surfaces of the hard twisted threads 125 as distinguished from having it distributed throughout the fibers of the threads as in the case when the sheets are treated by the ordinary so-termed wet method. As to this aspect of my invention, it is not necessary 130

that the adhesive material be applied to the textile material in the form of a powder. It may be applied equally well to the surface of the textile material in any other suitable manner, the essential thing being that the adhesive binder be located primarily on the surfaces of the threads. It will be understood that in the claims wherein I call for dry adhesive binder on the surfaces of the textile material, I mean that the adhesive binder is primarily on the surfaces as distinguished from being distributed throughout the fibers of the individual threads.

15 I preferably make the sheets in squares as this is a convenient shape and the metal plates 5 and 6 are made somewhat greater in dimensions so as to overlap them on all sides. This serves to take care of the widening out of the sheets when placed under compression and also to hold any bakelite which is squeezed out during the process.

20 My improved method, in addition to producing a material having properties superior to those of similar materials made by other methods possesses the further advantages when carried out with the use of an adhesive binder in powdered form that it can be carried out at a lower cost because 25 it saves the use of a solvent for the adhesive material, is simple to perform, and requires no expensive equipment.

30 What I claim as new and desire to secure by Letters Patent of the United States, is:—

35 1. The method of manufacturing a material of the character described from spinable textile woven fabric made from hard, twisted threads, and an adhesive binder, which comprises taking pieces of fabric and 40 stacking them one on another with a surface coating of the adhesive in dry form between them, subjecting the stack to pressure, and then heating the stack to fuse the adhesive binder.

45 2. The method of manufacturing a material of the character described from spinable textile woven fabric formed from hard, twisted threads, and an adhesive binder, which comprises taking pieces of fabric and 50 stacking them one on another with a surface coating of the adhesive in dry form between them, the warp of successive sheets being laid at a right angle to each other, sub-

jecting the stack to pressure, and then heating the stack to fuse the adhesive binder. 55

3. The method of manufacturing an indurated material from spinnable textile woven fabric made from hard, twisted threads, and phenolic condensation product which comprises stacking pieces of the woven 60 material one on another with a thin surface layer of dry phenolic condensation product between them, subjecting the stack to pressure, and then heating the stack while held under pressure to fuse the phenolic 65 condensation product.

4. The method of manufacturing a material of the character described from spinnable textile woven fabric made from hard, twisted threads and an adhesive binder, 70 which comprises taking pieces of fabric and stacking them one on another with a surface coating of the adhesive in dry form between them, subjecting the stack to pressure, heating the stack while held under pressure to 75 fuse the adhesive binder, and then cooling the resulting product while still under pressure.

5. The method of manufacturing an article of the character described from a textile 80 material comprising hard, twisted threads, and an adhesive binder, which comprises forming a stack from pieces of the material with dry adhesive binder located primarily on the surfaces of the pieces, subjecting the 85 stack to pressure, and then heating the stack while under pressure to fuse the adhesive binder whereby in the finished article the fibres of the hard, twisted, textile material are maintained in direct engagement with 90 each other by the surrounding adhesive material.

6. An indurated article comprising a plurality of pieces of textile material of hard twisted threads, said pieces being in close 95 proximity one with another, and a hard dry binding material extending through the interstices between the threads without saturating the threads, which binding material binds said threads together and holds the individual fibers of the threads closely compressed into direct contact with each other. 100

In witness whereof, I have hereunto set my hand this 12th day of August, 1921.

EMILE J. GUAY.